

1

3,268,311

### STABILIZED DISTILLATE HYDROCARBON FUEL OIL COMPOSITIONS

Roy L. Allen, Gresford, Wrexham, North Wales, and James H. T. Brook, Rockferry, Birkenhead, England, assignors to Shell Oil Company, New York, N.Y., a corporation of Delaware

No Drawing. Filed Dec. 3, 1962, Ser. No. 241,516  
Claims priority, application Great Britain, Jan. 25, 1962, 2,850/62

4 Claims. (Cl. 44—72)

This invention relates to liquid hydrocarbon fuels and in particular to distillate fuel oils, and is especially concerned with distillate fuel oils containing thermally or catalytically cracked products. By distillate fuel oil is meant a normally liquid mineral oil of which at least 98% volume can be distilled at a temperature not greater than 400° C. at atmospheric pressure, and having an ash of not more than 0.01% weight. It is an object of this invention to improve the stability of such fuel oils, i.e., to reduce their tendency to sludge deposition on storage for long periods.

According to the present invention a fuel oil composition comprises a distillate fuel consisting of up to 90% of a distillate fraction of a crude oil and 10% or more of a thermally or catalytically cracked product, and a small amount of one or more thiuram disulfides having on each nitrogen atom at least one substituent alkyl group of 5 or more carbon atoms.

These thiuram disulfides have been found to reduce substantially the tendency for sludge deposition of fuel oils and are greatly superior in this respect to other additives for the purpose, even closely related compounds such as alkyl substituted thiuram disulfides containing less than 5 carbon atoms per alkyl group, and alkyl and other substituted dithiocarbamates, as will be shown hereinafter.

To summarize, the thiuram disulfides which are useful in accordance with this invention are those having the formula



wherein R<sub>1</sub> is an alkyl radical having from 5 to 18 carbon atoms per molecule and R<sub>2</sub> is selected from the group consisting of hydrogen or alkyl radicals having from 1 to 18 carbon atoms per molecule. The thiuram disulfides which are most effective, however, are those containing four alkyl substituents on the two nitrogen atoms of the molecule. In the foregoing generic structural formula, both R<sub>1</sub> and R<sub>2</sub>, which are independently selected, are preferably alkyl radicals having from 5 to 18 carbon atoms per molecule. Tetra-N-alkyl-substituted thiuram disulfides in which the alkyl groups are the same are still further preferred. The thiuram disulfides with which the invention is concerned are readily made by oxidation of the corresponding dithiocarbamic acid with iodine.

The additive has been found to be effective in concentrations from 0.1 to 50 millimoles per liter of fuel. Surprisingly, a concentration range of from about 0.25 to 10 millimoles per liter has been found to give generally more effective results, and a range of from about 0.5 to about 5 millimoles per liter is still more effective and is therefore preferred.

This invention is particularly applicable to blended distillate fuels containing thermally or catalytically cracked products, which blends are exceptionally prone to sludge or sediment deposition, and which may block the filters or orifices of equipment used to burn the fuel. It appears that minor constituents of the various components of the blend interact with each other to produce an amount of sludge much greater than would be expected from the

2

sludging tendencies of each component taken separately, one example of such a distillate fuel blend is a diesel engine fuel blend comprising 50% of a straight run distillate and 50% of a catalytically cracked product. However, it is to be understood that 100% catalytic cracked products are not to be excluded since, as will be shown hereinafter, reduction of sludge deposition in these products is also achieved by the additives of the present invention. All these products contain sulfur compounds, often in the form of mercaptans, and also various olefinic and aromatic compounds.

The following are examples of fuels in accordance with this invention which have been made and tested:

#### EXAMPLE I

A light catalytically cracked cycle oil (LCCCO) having a mercaptan content of 538 parts per million measured as sulfur and 129 parts per million total nitrogen, which base fuel contains tetraamyl thiuram disulfide at a concentration of 10 millimoles per liter of fuel.

#### EXAMPLE II

Equal parts of a LCCCO and a light straight run gas oil (LSRGO), having a mercaptan content of 376 parts per million measured as sulfur and 116 parts per million total nitrogen, which base fuel contains tetraamyl thiuram disulfide at a concentration of 10 millimoles per liter of fuel.

#### EXAMPLE III

Equal parts of a LCCCO and a medium straight run gas oil (MSRGO) having 124 parts per million basic nitrogen and 148 parts per million total nitrogen which base fuel contains tetraamyl thiuram disulfide at a concentration of:

- (a) 1 millimole per liter of fuel.
- (b) 10 millimoles per liter of fuel.

The improved quality of these fuels can be assessed by determining the amount of sludge developed in the fuel after it has been stored in cans under natural conditions for a known period. The fuel is filtered through a special paper having a controlled pore size of 0.45 micron, and the sludge is washed with light petroleum naphtha (60°—80° C. b.p.). The paper and sludge is then dried at 103° C. for one hour, cooled and weighed. The weight of the paper filter, previously determined after drying for one hour at 103° C., is deducted to obtain the weight of the suspended sludge in the fuel. Sludge adhering to the can is dissolved in ethanol, the solvent is removed by evaporation, the sludge is dried at 103° C. and weighed. These quantities are then summed to give the amount of developed sludge in milligrams per 100 milliliters of fuel. In addition to this sludge, a further quantity can be precipitated by diluting the filtered fuel with 10 parts by volume of light petroleum naphtha (30°—40° C. b.p.). This is then allowed to stand overnight and is then determined in the same way as the suspended sludge. This additional sludge has a chemical composition similar to that of the suspended sludge, and may be either the precursor of the fully formed sludge, or a fully formed sludge which remains dissolved in the fuel only because of the aromaticity of the fuel; when the aromaticity is decreased by dilution the sludge precipitates.

In the following tables, which further illustrate the present invention, the sludging tendency of the fuel is taken as the sum of the three types of sludge hereinbefore described.

Table I shows the results of tests carried out on Examples I and II, and on the base fuels used in these examples containing substituted dithiocarbamates in place of tetraamyl thiuram disulfide, the results are expressed as a percentage of the control, i.e., fuel without additive.

The blends were stored by the filtration and ethanol procedure previously described.

Table I

| Example I base fuel:                                                 | Sludging tendency percent | 5  |
|----------------------------------------------------------------------|---------------------------|----|
| Without additive                                                     | 100                       |    |
| With 10 millimoles tetraamyl thiuram disulfide/liter                 | 22                        |    |
| With 10 millimoles piperidinium pentamethylene dithiocarbamate/liter | 62                        | 10 |
| With 10 millimoles dibutyl ammonium dibutyl dithiocarbamate/liter    | 46                        |    |
| Example II base fuel:                                                | 15                        |    |
| Without additive                                                     | 100                       |    |
| With 10 millimoles tetraamyl thiuram disulfide/liter                 | 14                        |    |
| With 10 millimoles piperidinium pentamethylene dithiocarbamate/liter | 46                        | 20 |
| With 10 millimoles dibutyl ammonium dibutyl dithiocarbamate/liter    | 43                        |    |

It is evident from the above table that the tetraalkyl thiuram disulfide of this invention is much more effective than the substituted dithiocarbamates.

Further tests were carried out to illustrate the superiority of tetraamyl thiuram disulfide, as an additive for reducing sludge deposition in fuel oils, over tetraalkyl substituted thiuram disulfide containing shorter (i.e., less than 5 carbon atoms) alkyl chains. The results are shown in Table II.

Table II

(STORAGE TEMPERATURE 25° C.)

| Storage Period |                                                | Developed Sludge | Precipitated Sludge | Total Sludge |
|----------------|------------------------------------------------|------------------|---------------------|--------------|
| 3 months.      | Example I Base Fuel without additive           | 6.2              | 8.5                 | 14.7         |
|                | Example I Base Fuel plus 10 millimoles/liter:  |                  |                     |              |
|                | Tetramethyl thiuram disulfide                  | 52.0             | 14.2                | 66.2         |
|                | Tetraethyl thiuram disulfide                   | 8.2              | 1.7                 | 9.9          |
|                | Tetrabutyl thiuram disulfide                   | 10.9             | 4.5                 | 15.4         |
|                | Tetraamyl thiuram disulfide                    | 1.7              | 1.6                 | 3.3          |
| 3 months.      | Example II Base Fuel without additive          | 4.2              | 2.5                 | 6.7          |
|                | Example II Base Fuel plus 10 millimoles/liter: |                  |                     |              |
|                | Tetraethyl thiuram disulfide                   | 5.7              | 0.5                 | 6.2          |
|                | Tetrabutyl thiuram disulfide                   | 1.9              | 5.2                 | 7.1          |
|                | Tetraamyl thiuram disulfide                    | 0.3              | 0.6                 | 0.9          |
| 6 months.      | Example II Base Fuel without additive          | 7.6              | 3.7                 | 11.3         |
|                | Example II Base Fuel plus 10 millimoles/liter: |                  |                     |              |
|                | Tetraethyl thiuram disulfide                   | 13.7             | 1.5                 | 15.2         |
|                | Tetrabutyl thiuram disulfide                   | 11.0             | 3.3                 | 14.3         |
|                | Tetraamyl thiuram disulfide                    | 1.6              | 1.8                 | 3.4          |

Table III shows the results when the fuels of Example III were stored for different known periods at a temperature of 25° C., and then tested for sludge deposition by the described methods.

In addition to the above, it will be recognized that the N-alkyl substituted thiuram disulfide compounds with which the invention is concerned can be used in fuel oil compositions containing hydrogen treated petroleum frac-

Table III

| Storage Period      | 3 Months                         |              |              | 6 Months                         |              |              | 9 Months                         |              |              | 12 Months                        |              |              |
|---------------------|----------------------------------|--------------|--------------|----------------------------------|--------------|--------------|----------------------------------|--------------|--------------|----------------------------------|--------------|--------------|
|                     | Fuel of Example without Additive | Example IIIa | Example IIIb | Fuel of Example without Additive | Example IIIa | Example IIIb | Fuel of Example without Additive | Example IIIa | Example IIIb | Fuel of Example without Additive | Example IIIa | Example IIIb |
| Developed Sludge    | 6.1                              | 0.1          | 3.2          | 6.9                              | 0.8          | 2.5          | 7.7                              | 1.2          | 6.3          | 11.6                             | 1.7          | -----        |
| Precipitated Sludge | 3.2                              | 0.0          | 1.4          | 4.0                              | 1.4          | 1.2          | 4.5                              | 2.0          | 2.8          | 6.3                              | 1.3          | -----        |
| Total Sludge        | 9.3                              | 0.1          | 4.6          | 10.9                             | 2.2          | 3.7          | 12.2                             | 3.2          | 9.1          | 17.9                             | 3.0          | -----        |

Other examples of fuels in accordance with the invention are as follows:

## EXAMPLE IV

A light catalytically cracked gas oil containing 0.99% wt. sulfur and 190 parts per million (p.p.m.) nitrogen and containing 5 millimoles per liter (basis gas oil) of N,N'-diethyl-N,N'-dioctyl thiuram disulfide.

tions, which may be either straight run or cracked fractions, and which have been treated with hydrogen for any number of purposes such as removal of metallic contaminants, reduction or removal of sulfur compounds, reduction of nitrogen compounds, or to adjust physical properties such as molecular weight, viscosity or pour point.

4  
EXAMPLE V

A mixture of 60% by volume straight run gas oil containing 0.17% wt. sulfur and 72 p.p.m. nitrogen and 40% by volume catalytically cracked gas oil containing 1.36% wt. sulfur and 380 p.p.m. nitrogen and containing per liter of gas oil mixture 1 millimole per liter of tetrahexadecanyl thiuram disulfide.

## EXAMPLE VI

A mixture of straight run and cracked distillate hydrocarbons containing 0.5 millimole per liter of tetradecanyl thiuram disulfide, the mixture having the following composition and component properties:

| Component Properties          | Hydro-treated Light Straight Run Distillate | Cat. Cracked Gas Oil | Straight Run Gas Oil |
|-------------------------------|---------------------------------------------|----------------------|----------------------|
|                               | Percent by Volume                           |                      |                      |
|                               | 15                                          | 50                   | 35                   |
| Gravity, ° API                | 40.4                                        | 28.8                 | 32.9                 |
| Mercaptan Sulfur, g./100 cc.  | 0.0005                                      | 0.0008               | 0.0067               |
| Thiophenol Sulfur, g./100 cc. | 0.0004                                      | 0.0004               | 0.0072               |
| Disulfide Sulfur, g./100 cc.  | 0.0002                                      | 0.0052               | 0.016                |
| Total Sulfur, percent wt.     | 0.155                                       | 0.92                 | 0.90                 |
| ASTM Distillation, ° F.:      |                                             |                      |                      |
| Initial Boiling Point         | 386                                         | 444                  | 456                  |
| 10% Recovered                 | 414                                         | 480                  | 528                  |
| 50% Recovered                 | 488                                         | 534                  | 574                  |
| 90% Recovered                 | 500                                         | 596                  | 610                  |
| End Point                     | 534                                         | 640                  | 632                  |

We claim as our invention:

1. A liquid hydrocarbon distillate fuel oil composition containing at least 10% by volume of normally liquid hydrocarbons produced from the cracking of petroleum hydrocarbons and from 0.1 to 10 millimoles per liter of said composition of a thiuram disulfide corresponding to the structural formula



wherein  $R_1$  is an alkyl radical having from 5 to 18 carbon atoms per molecule and  $R_2$  is selected from the group consisting of hydrogen and alkyl radicals having from 1 to 18 carbon atoms per molecule.

2. A liquid hydrocarbon distillate fuel oil composition containing at least 10% by volume of normally liquid hydrocarbons produced from the cracking of petroleum hydrocarbons and from 0.25 to 10 millimoles per liter of said composition of a thiuram disulfide corresponding to the structural formula



wherein  $R_1$  and  $R_2$  are independently selected alkyl radicals having from 5 to 18 carbon atoms per molecule.

3. A liquid hydrocarbon distillate fuel oil composition containing at least 10% by volume of normally liquid hydrocarbons produced from the cracking of petroleum hydrocarbons and from about 0.5 to about 5 millimoles per liter of said composition of a thiuram disulfide corresponding to the structural formula



10 wherein  $R_1$  and  $R_2$  are independently selected alkyl radicals having from 5 to 18 carbon atoms per molecule.

4. A liquid hydrocarbon distillate fuel oil composition containing at least 10% by volume of normally liquid hydrocarbons produced from the cracking of petroleum hydrocarbons and from 0.1 to 10 millimoles per liter of said composition of tetraamyl thiuram disulfide.

References Cited by the Examiner

UNITED STATES PATENTS

|           |         |       |       |            |
|-----------|---------|-------|-------|------------|
| 2,160,851 | 6/1939  | Faust | ----- | 44—72      |
| 2,268,382 | 12/1941 | Cloud | ----- | 44—76 X    |
| 2,681,316 | 6/1954  | Harle | ----- | 252—47.5   |
| 2,691,632 | 10/1954 | Harle | ----- | 252—47.5 X |

DANIEL E. WYMAN, Primary Examiner.

C. O. THOMAS, J. E. DEMPSEY, Y. M. HARRIS,  
Assistant Examiners.